

Dec. 29, 1936.

E. H. TRUSSELL

2,065,769

COATED OBJECT AND PROCESS OF MAKING THE SAME

Filed March 6, 1934

FIG. 1.



FIG. 2.



Inventor

*Emory H. Trussell.*

By *Stone, Boyd & Mack.*  
Attorneys

## UNITED STATES PATENT OFFICE

2,065,769

COATED OBJECT AND PROCESS OF  
MANUFACTURING THE SAMEEmory H. Trussell, Newark, N. J., assignor to  
Beckwith-Chandler Company, Newark, N. J., a  
corporation of New Jersey

Application March 6, 1934, Serial No. 714,302

11 Claims. (Cl. 91—68)

This invention relates to coated objects and to the method of providing surfaces with an improved finish for decorative or protective purposes. The improvement pertains generally to the surface characteristics of lacquer coatings.

Heretofore in the production of a smooth finish on rough surfaces, such as wood or metal with file marks, pit holes, etc., with cellulose ester lacquers and particularly cellulose nitrate lacquers serious difficulties arose from the use of the strong solvents of the nitrate lacquer in that they dissolve the undercoats which were used to build up the priming and filling coats for the rough object. The undercoats become swelled and more or less raised out of the imperfections in the surface and on the evaporation of the solvent draw back down to an irregular film showing indentations for each of the rough spots in the surface of the object coated. Furthermore in the building of a quick air drying finish on rough objects of this nature it is very desirable to use undercoats which not only stick to the surface of the object and fill the imperfections in the surface, but also dry hard quickly principally by the evaporation of solvents. For this purpose primers and surfacers built around a cellulose ester base, and particularly nitro-cellulose base, have been and are used very extensively. Now when this type of undercoat is used and the finish or color coat of cellulose ester lacquer are thereafter applied, not only is there a dissolving of the undercoat which results in the swelling and pulling out of the imperfections in the surface of the object coated but also when the solvents evaporate the entire surface takes on a soaked in or microscopic pitted appearance due probably to a complete amalgamation of the two films. In order to overcome this appearance, it is necessary to rub and polish the surface, when it has thoroughly dried, with an abrasive and polishing material.

The aforementioned difficulties are somewhat overcome in the production of cellulose ester finishes at present, by the use of undercoats which are of the oil base or drying oil base, and synthetic resin type base baked on to the surface at varying elevated temperatures in ovens and for varying periods of time. This somewhat eliminates the soaking in and swelling trouble but still there is enough softening of the undercoats to still yield a finished surface of the cellulose ester lacquer that shows roughness and unevenness undesirable for a good decorative finish.

This unevenness can be and is removed by the

rubbing and polishing operation after the lacquer has dried thoroughly.

In the present invention the above mentioned difficulties due to the dissolving of one coat by the application of succeeding coats are overcome by using as a finishing coat of lacquer over a cellulose ester lacquer, a composition containing as its base cellulose ethers such as benzyl and ethyl cellulose which are soluble in coal tar hydrocarbons such as benzene, toluene, xylene and high flash solvent naphtha or mixtures of these hydrocarbons with relatively small proportions of cellosolve (generally known to be mono-ethyl ether of ethylene glycol) or one or more alcohols such as butanol, the amyl alcohols, etc. These hydrocarbon materials or the aforesaid mixtures are not solvents for the cellulose ester films and by taking advantage of this fact the cellulose ether coatings may be applied over a base of nitrocellulose or cellulose ester undercoat without soaking in or softening to the point that the base coat is drawn from imperfections in the surface to be coated.

To more specifically explain the present invention, the surface of the object to be coated may be coated with primer and filler of nitrocellulose base, and sanded smoothly when dried to get a perfectly level or smooth surface. Then a finished decorative coat or coats of benzyl cellulose base lacquer are applied. The resulting finish when properly formulated for the method of application will dry to a smooth even surface not showing any of the imperfections in the surface coated and not having the soaked in or micro pitted appearance. If, however, the same nitrocellulose base had been used in the finished coat of lacquer, the solvents would have dissolved the nitrocellulose undercoat and the resulting dried film would have been rough and uneven with a soaked in or micro pitted appearance.

In certain instances, the surface of the object to be coated may first be primed with other types of material such as drying oil base or synthetic resin base material. Then after they are sufficiently dried an intermediate coating or filling coat of cellulose ester such as cellulose nitrate is applied, thoroughly dried, sanded and a top coating of the cellulose ether lacquer applied as a finish coat. By this method the same objects of the invention are accomplished.

An object of the present invention is to provide a process by which solid objects are produced having smooth or glossy finishes by the use of lacquer materials.

A further object is to provide coated articles, the surfaces of which have a finish that is practically free from imperfections that are ordinarily encountered in lacquer coatings that have 5 not received a rubbing or polishing treatment.

From the aforementioned facts, it can be seen that a still further object of my invention is to produce a quick drying finish for wood, metal, and like objects, as well as fibrous sheets. For 10 the purposes of the present invention, cloth or felt or other sheet materials may be considered solid objects. The finish is smooth or glossy as may be desired without the laborious task of rubbing and polishing the final coat. The 15 success of my invention lies in the fact that a cellulose ether coating, and more specifically a benzyl or ethyl cellulose coating, containing a solvent mixture that does not dissolve the preceding coat which is of a cellulose ester base, 20 more specifically cellulose nitrate or acetate, when the finishing coat is superimposed on the cellulose ester coating.

The present invention is illustrated in the accompanying drawing, in which:

25 Fig. 1 is a sectional view showing a supporting element with a surface having an inner coating of nitrocellulose or cellulose ester base material and an outer coating of cellulose ether base material; and.

30 Fig. 2 is a sectional view showing a supporting element with a surface having a primer coat of oil base or oil and resin base material, an intermediate coat of nitrocellulose or cellulose ester base material and an outer coat of cellulose ether base material.

35 The various layers employed may be prepared from pigmented or from clear liquid compositions. The rate of evaporation of the solvents used can be regulated, in the well known manner, from a very rapid rate, like the fastest drying lacquers, to a medium speed comparable to that of the more rapidly drying enamels.

The various ingredients employed in the lacquers are selected to provide compatible mixtures as is understood in the art. For instance, 40 ethyl cellulose is considered compatible with natural resins such as damar as well as both the phenol aldehyde and the resins of the alkyd type including for instance glycerol phthalate 45 synthetic types, both pure and modified. On the other hand, the benzyl cellulose is not considered compatible with the majority of the natural resins such as damar, but it is considered compatible with those of the synthetic types 50 mentioned above. Rapid developments have been and are being made in the field of synthetic resins. Excellent results have been obtained with lacquers containing combinations of benzyl cellulose and glycerol phthalate synthetic 55 resins. I have prepared films that are dry and clear and with very bright glossy surfaces, from combinations in which the proportions of cellulose ether to glycerol phthalate resins varied from equal parts of cellulose ether and resin to 60 cases where four or five parts of the resin to one part of cellulose ether were present.

65 Other alkyd resins that may be mentioned as useful are those formed by the combination of polyhydric alcohols including glycerine with an aliphatic acid such as maleic as well as phthalic mentioned above. Combinations of these acids including also benzoic with other aliphatic acids such as oleic, linoleic and so forth, are also useful in the production of resins from polyhydric 70 alcohols.

It is understood that other types of resins such as ester gum also give highly satisfactory results particularly in the less expensive type of finish.

The following examples illustrate the process 5 of the present invention:

*Example 1.*—A composition such as the following is applied to a metal or other surface as a priming or filling coat:

|                                                                                                                                                                                                                                                     | Parts 10 |
|-----------------------------------------------------------------------------------------------------------------------------------------------------------------------------------------------------------------------------------------------------|----------|
| Talc                                                                                                                                                                                                                                                | 150      |
| Zinc oxide                                                                                                                                                                                                                                          | 150      |
| Dry nitrocellulose                                                                                                                                                                                                                                  | 100      |
| Tricresyl phosphate                                                                                                                                                                                                                                 | 35       |
| Blown castor oil                                                                                                                                                                                                                                    | 40 15    |
| Solvent mixture composed of proper balance of ester solvents (such as ethyl, butyl, or amyl acetates) alcohols (such as butanol, ethanol, etc.) and hydrocarbons (such as toluene, xylene, or even portions of fast evaporating petroleum naphthas) | 20 1100. |

It is understood that the hydrocarbons in the above formula are included merely as diluents in the well known manner and proportions. The 25 proportions are limited only to such an extent as will cause no precipitation of the nitrocellulose material.

The composition of this undercoat may be varied widely as long as it adheres to the metal 30 surface, fills the imperfections and is built on a nitrocellulose, or cellulose ester base insoluble in toluene, xylene, etc., or mixtures of these hydrocarbons and alcohols containing a major portion of hydrocarbon. After this undercoat 35 is dried, it is rubbed, by which is meant sanded smooth with fine abrasives. Then a finish coat of the following composition may be applied:

|                                | Parts 40 |
|--------------------------------|----------|
| Antimony oxide                 | 230      |
| Plastic alkyd resin            | 230      |
| Benzyl cellulose low viscosity | 50       |
| Xylene                         | 540      |
| Butanol                        | 85 45    |

The composition of this finished coat may be varied between wide limits as long as it is built around a cellulose ether base and is composed of ingredients that are compatible and soluble in the solvent mixture used. This finish may be 50 made in various colors or clear.

*Example 2.*—As another example of my invention, I may use as a priming coat for a metal surface a composition of a drying oil type or oxidizing synthetic resin type as follows:

|                                                                                                                                                                                                                                     | Parts  |
|-------------------------------------------------------------------------------------------------------------------------------------------------------------------------------------------------------------------------------------|--------|
| Pigment—mixture of iron oxide and inert or any suitable mixture known to one familiar with the art                                                                                                                                  | 100 60 |
| Fixed vehicle—composed of mixture of drying oils such as linseed and China-wood oils with resins such as East India resin, ester gum, etc. properly blended and heat treated to give desired drying time familiar to one in the art | 65     |
| Thinner—usually petroleum distillate or mixture thereof with turpentine                                                                                                                                                             | 50-60  |
| Oxidizing synthetic resin types of undercoat:                                                                                                                                                                                       | 70     |
| Pigment of suitable mixture                                                                                                                                                                                                         | 100    |
| Resin such as of the alkyd type                                                                                                                                                                                                     | 40     |
| Solvent such as xylene or mixed solvent suitable for purpose                                                                                                                                                                        | 100 75 |

2. A process of manufacturing a coated metal object, which process comprises applying a cellulose ester lacquer to a surface of said object, drying and rubbing the coating formed on said object, applying a cellulose ether lacquer to the said coating, the said cellulose ether lacquer containing a hydrocarbon solvent material that is not a solvent for the cellulose ester, and permitting the cellulose ether lacquer coating to dry to thereby form a smooth, finished surface.
3. A process of manufacturing a coated metal object, which process comprises applying to a surface of said object a priming coat, then applying a cellulose ester lacquer coating and finally a cellulose ether lacquer coating, the said cellulose ether lacquer applied to said cellulose ester lacquer coating containing hydrocarbon solvent material that is not a solvent for the cellulose ester, thereby forming a smooth, finished surface.
4. A process of manufacturing a coated metal object, which process comprises applying to a surface of said object a coating containing a cellulose plastic that is not dissolved by low boiling hydrocarbons alone, applying directly to the surface of said coating a solution of cellulose ether in a solvent containing low boiling hydrocarbon liquid in such proportion that the solvent does not soften the said cellulose plastic coating, and permitting the said solution to dry on the said first coating to thereby form a smooth, finished surface.
5. A process of manufacturing a coated metal object, which process comprises applying the following composition to a surface of the said object to form a coating:

| Parts by weight     |      |
|---------------------|------|
| Talc                | 150  |
| Zinc oxide          | 150  |
| 40 Nitrocellulose   | 100  |
| Tricresyl phosphate | 35   |
| Blown castor oil    | 40   |
| Solvent             | 1100 |

45 applying to the coating resulting from the above application the following composition:

| Parts by weight                   |     |
|-----------------------------------|-----|
| Antimony oxide                    | 230 |
| Plastic alkyd resin               | 230 |
| Benzyl cellulose of low viscosity | 50  |
| Xylene                            | 540 |
| Butanol                           | 85  |

55 and permitting drying of the resulting object to form a smooth, finished surface.

6. A process of manufacturing a coated metal object, which process comprises applying to a surface of the said object a priming coat containing 100 parts by weight of pigment and 100 to 140 parts by weight of a mixture of binder material and solvent, applying to the priming coat resulting from the above application the following composition:

| Parts by weight     |      |
|---------------------|------|
| Talc                | 150  |
| Zinc oxide          | 150  |
| Nitrocellulose      | 100  |
| Tricresyl phosphate | 35   |
| 70 Blown castor oil | 40   |
| Solvent             | 1100 |

75 applying to the surface of the coating resulting from the application of the last-named composition the following composition:

| Parts by weight                   |     |
|-----------------------------------|-----|
| Antimony oxide                    | 230 |
| Plastic alkyd resin               | 230 |
| Benzyl cellulose of low viscosity | 50  |
| Xylene                            | 540 |
| Butanol                           | 85  |

and permitting drying of the resulting object to form a smooth, finished surface.

7. A process of manufacturing a coated metal object, which process comprises applying to a surface of the said object a coating containing cellulose plastic that is not dissolved by low-boiling hydrocarbons alone, applying directly to the said coating a cellulose ether lacquer, the solvent in which contains low-boiling coal tar hydrocarbon liquid material in predominating proportions as compared with other constituents of the said solvent, thereby inhibiting softening of the said coating containing the said cellulose plastic; and permitting drying of the resulting object to form a smooth, finished surface.

8. An article of manufacture produced by the process of claim 1, the said article comprising a metal supporting element having a plurality of plastic coatings thereon including an inner coating of cellulose ester-containing material and a superposed outside coating of cellulose ether-containing material, the latter coating having a uniformly smooth surface characterized by being free from that pitted appearance resulting from the application of cellulose ester coating compositions to inner coatings of cellulose ester.

9. An article of manufacture produced by the process of claim 3, the said article comprising a metal supporting element having a plurality of coatings thereon including a priming coat, an intermediate coating of cellulose ester-containing material and a superposed outside coating of cellulose ether-containing material, the latter 40 coating having a uniformly smooth surface characterized by being free from that pitted appearance resulting from the application of coatings of cellulose ester to inner coatings of cellulose ester.

10. An article of manufacture produced by the process of claim 5, the said article comprising a metal supporting element having a plurality of coatings thereon including an inner coating resulting from the application of substantially 50 the following composition:

| Parts by weight     |      |
|---------------------|------|
| Talc                | 150  |
| Zinc oxide          | 150  |
| Nitrocellulose      | 100  |
| Tricresyl phosphate | 35   |
| Blown castor oil    | 40   |
| Solvent             | 1100 |

and a superposed outside coating resulting from the application of substantially the following composition:

| Parts by weight                   |     |
|-----------------------------------|-----|
| Antimony oxide                    | 230 |
| Plastic alkyd resin               | 230 |
| Benzyl cellulose of low viscosity | 50  |
| Xylene                            | 540 |
| Butanol                           | 85  |

the latter coating having a uniformly smooth surface characterized by being free from that pitted appearance resulting from the application of coatings of cellulose ester on inner coatings of cellulose ester.

Either of these materials or suitably varied compositions of their nature are applied to the metal surface permitted to dry for the required length of time known from the formulae used, 5 and then a surfacing coat of nitrocellulose such as the one mentioned above is applied over it to fill imperfections in the metal and act as a base for the top coat of cellulose ether lacquers such as the one mentioned above.

10 It will be obvious to one familiar with the art that numerous compositions of the aforesaid nature are available and suitable for the purpose intended and that such procedure of building a finish is readily adaptable to other 15 types of rigid surfaces such as wood, press board, and materials of that nature.

For example, other types of cellulose ether lacquers are given below as follows:

20 *Benzyl cellulose base solution 39301*

|                                | Parts |
|--------------------------------|-------|
| Benzyl cellulose—low viscosity | 100   |
| Xylol                          | 300   |
| 25 Butanol                     | 30    |

*Clear benzyl cellulose lacquer*

|                                                                                                         | Parts |
|---------------------------------------------------------------------------------------------------------|-------|
| 39301 base                                                                                              | 50    |
| 30 Alkyd resin solution composed of 1 part of what is known in the trade as rezyl 1102 and 1 part xylol | 96    |
| Xylol                                                                                                   | 45    |
| 35 Butyl alcohol (butanol)                                                                              | 11    |

*Clear benzyl cellulose lacquer*

|                  | Parts |
|------------------|-------|
| Benzyl cellulose | 100   |
| Rezyl 1102       | 300   |
| 40 Xylene        | 835   |
| Butanol          | 90    |
| Butyl cellosolve | 5     |

It will be noted that there is a small quantity 45 of butyl cellosolve (mono butyl ether of ethylene glycol) present in this formula. This material, while a solvent for the whole film, when used in small quantities does not appreciably dissolve the undercoat and materially improves the compatibility of the resin and ether as well as helps the flow of the finished coat.

*White benzyl cellulose lacquer*

|                     | Parts |
|---------------------|-------|
| 55 Antimony oxide   | 100   |
| Rezyl 1102          | 100   |
| Xylol               | 100   |
| Butanol             | 10    |
| 60 Butyl cellosolve | 22    |
| 39301 base          | 110   |
| Xylol               | 119   |
| Butanol             | 13    |

*Colored benzyl cellulose lacquer*

|                      | Parts |
|----------------------|-------|
| Chrome green pigment | 40    |
| Rezyl 1102           | 150   |
| Benzyl cellulose     | 75    |
| 70 Xylene            | 660   |
| Butanol              | 63    |

This formula produces a green lacquer and demonstrates the use of a reduced quantity of resin in proportion to the benzyl cellulose.

*Clear lacquer*

|                                               | Parts |
|-----------------------------------------------|-------|
| Benzyl cellulose                              | 100   |
| Alkyd resin known in the trade as Amberol 801 | 150   |
| Dibutyl phthalate                             | 30    |
| Xylol                                         | 765   |
| Butanol                                       | 85    |
| Butyl cellosolve                              | 8½    |

10 This formula demonstrates the use of the benzyl cellulose lacquer in the clear state and also shows a combination of this ether with a synthetic plasticizer and hard synthetic resin.

*Clear ethyl cellulose lacquer*

|                     | Parts |
|---------------------|-------|
| Ethyl cellulose     | 100   |
| Damar gum (dewaxed) | 100   |
| Dibutyl phthalate   | 30    |
| Toluene             | 300   |
| Xylene              | 400   |
| 25 Butanol          | 75    |

25 This formula shows the use of ethyl cellulose with the natural resin damar and dibutyl phthalate plasticizer. The combination makes an excellent clear finish for decorative purpose.

*Colored ethyl cellulose lacquer*

|                                                 | Parts |
|-------------------------------------------------|-------|
| Para red pigment                                | 40    |
| Ethyl cellulose                                 | 100   |
| Alkyd resin known in the trade as Lewisol L-500 | 200   |
| Dibutyl phthalate                               | 25    |
| Xylene                                          | 770   |
| 35 Butanol                                      | 85    |
| Butyl cellosolve                                | 5     |

40 The above formula shows the further use of ethyl cellulose in a red lacquer, making use of an alkyd type resin and synthetic plasticizer.

45 These are only typical formulae and numerous other combinations of resins in the alkyd class as well as the phenol aldehyde class can be used.

50 Cellulose ether coatings of the type set forth have excellent levelling properties and are in general very alkali and water resistant. In the application of cellulose ether lacquers to the process of the present invention, it is distinctly demonstrated that they do not soak into or soften undercoatings prepared from cellulose esters including cellulose nitrate or cellulose acetate but on the contrary leave such undercoatings unaffected and thereby dry to a smooth or glossy hard perfect finish.

55 The proportions of ingredients in the formulae given herein, are in parts by weight.

It is to be understood that the hydrocarbon solvent material for the cellulose ether lacquer, referred to in the claims, is not considered a 60 solvent for cellulose esters at those temperatures at which paints and lacquers are ordinarily applied for coating purposes.

What I claim is:

65 1. A process of manufacturing a coated metal object, which process comprises applying to a surface of said object a cellulose ester composition to form a solid film that is not dissolved by low-boiling hydrocarbons alone, applying directly to the surface of said film a solution of cellulose ether in a solvent containing low-boiling hydrocarbon liquid in such proportion that the solvent does not soften the said film, and permitting the said solution to dry on the said film to thereby form a smooth, finished surface.

11. An article of manufacture produced by the process of claim 6, the said article comprising a metal supporting element having a plurality of coatings thereon including a priming coat, an intermediate coating resulting from the application of substantially the following composition:

Parts by weight

|                     |      |
|---------------------|------|
| Talc                | 150  |
| Zinc oxide          | 150  |
| 10 Nitrocellulose   | 100  |
| Tricresyl phosphate | 35   |
| Blown castor oil    | 40   |
| Solvent             | 1100 |

15 and a superposed outside coating resulting from

the application of substantially the following composition:

|                                   | Parts by weight |
|-----------------------------------|-----------------|
| Antimony oxide                    | 230             |
| Plastic alkyd resin               | 230             |
| Benzyl cellulose of low viscosity | 50              |
| Xylene                            | 540             |
| Butanol                           | 85              |

the latter coating having a uniformly smooth 10 surface characterized by being free from that pitted appearance resulting from the application of coatings of cellulose ester to inner coatings of cellulose ester.

EMORY H. TRUSSELL. 15